

## UNITED STATES PATENT OFFICE.

BYRAMJI D. SAKLATWALLA, OF CRAFTON, PENNSYLVANIA.

## FERROUS ALLOY.

No Drawing.

Application filed August 26, 1922. Serial No. 584,552.

The present invention relates to ferrous alloys, and particularly to a ferrous alloy containing chromium and copper. The addition of chromium to ferrous metal containing carbon imparts to it great hardness. To combine increased ductility and dynamic strength with this property several alloying elements, such as nickel and molybdenum, either singly or in combination are at present added to steel together with the chromium. All such elements are costly and consequently unduly raise the manufacturing cost of the steel by their addition.

The disadvantage of high cost is obviated and chromium steels combining high tensile strength with remarkable ductility are produced by the addition of copper to them. The percentages of copper necessary to produce this result are low, so that the reduction of cost is attained, not only owing to the comparatively cheap price of copper, but also to the very small amount of copper used per ton of finished steel.

It has been found that an addition of copper, ranging from .15 to .50% to steel containing .3 to 3.50% chromium increases its ductility and toughness to a very remarkable extent. The presence of copper also does not interfere with any properties imparted to the steel by reason of its carbon and chromium contents. On the contrary, the copper content acts in an additive manner towards augmenting the tensile strength derived from the carbon and chromium contents, also increasing the ratio of elastic limit to tensile strength. Consequently, it is possible to obtain steels of widely different physical properties suitable for a wide range of purposes, by varying the combinations of percentages of carbon, chromium and copper in them. Also the presence of copper does not interfere in any way with the possibilities of heat treatment, thus allowing a latitude in the production of a variation of physical properties.

Such combinations of chromium and copper are useful in ferrous alloys, not only of the steel range, that is, containing carbon up to about 2%, but also in the cast iron ranges of carbon between 2 and 3.50%. Combinations of copper from .15 to .50% and chromium from .3 to 3.50% impart to cast iron properties of great hardness and strength, also the remarkable property of possessing this hardness and strength

higher temperatures, at the same time withstanding the action of oxidation at such temperatures.

The ferrous alloys of these chromium copper compositions besides showing the described physical properties, possess an extremely high degree of resistance to corrosion, not only in the hardened, but also in the annealed and natural states as cast, forged or rolled. Their resistance to mineral acid corrosion is especially remarkable. Also it is possible to produce the resistance necessary for a particular case by varying the chromium and copper contents. For instance, in the case of sulphuric and hydrochloric acids, the higher the copper content, the more resistive the alloy is to sulphuric and less to hydrochloric, and the higher the chromium content, the more resistive it is to hydrochloric and less to sulphuric acids. Also the resistance to corrosion is influenced by the carbon content, the higher the carbon, the less resistive is the alloy to corrosion. This disadvantage of the high carbon content can, however, be obviated by an increased silicon content up to about 1%, the effect of such a content of silicon being the same as though the high percentage of carbon were absent.

The silicon not only affects the non-corrosive properties of the alloy, but also its mechanical properties, such as hardness. The presence of silicon in the chromium-copper-ferrous alloy allows it to be more easily rolled and fabricated and imparts ductility to the metal.

Claims directed specifically to the inclusion of silicon in the applicant's chromium-copper-ferrous alloy are presented in applicant's copending application, Serial No. 704,633, filed April 7, 1924.

It is thus obvious that by the variation of percentages of chromium, copper, carbon and with the help of silicon a variety of ferrous alloys can be produced, which are non-corrosive to particular agencies in question, such as organic and mineral acids, mine waters, sea and fresh waters, atmospheric influences, and which are of the desired malleability, etc.

It has been found that steels containing from .3 to 1.25% of chromium and only .15 to .50% copper have very remarkable all-round non-corrosive properties, suitable for several purposes. This fact makes this

range of steels extremely useful in the arts, as they also possess remarkable physical properties of static and dynamic strength with high degree of ductility.

5 In making usual steels which can be rolled and machined, I prefer to use the minimum amounts of chromium and copper to give the desired characteristics. As above pointed out, by combining comparatively small 10 quantities of chromium and copper, the manufacturing cost can be kept to a minimum. There is also another important advantage in using the comparatively small amounts of chromium and copper specified, namely, that 15 the alloy is more reliable than when larger amounts of chromium and copper are employed. It is a generally recognized rule that the smaller the alloying elements in steel, the more reliable is the steel, and I 20 have found this to be true of a copper and chromium alloy steel. For the usual steels, I prefer to use about .4 to 1% of chromium and from .2 to .4% of copper. These 25 percentages are sufficient to give high tensile strength, considerable ductility and resistance to corrosion. These amounts of copper and chromium are low enough so that the alloy is very reliable. These comparatively small amounts of copper and 30 chromium give to the steel substantially the same resistance to corrosion as higher amounts of copper and chromium and a considerably greater resistance to corrosion than considerably greater amounts of copper and chromium used alone. They also 35 give better physical properties than larger amounts of copper and chromium mixed or larger amounts of copper alone or chromium alone. There is apparently a critical limit 40 of about one-half of 1% for copper when added to a low chrome steel, that is, a chrome steel having not more than about 2 or 3% of chromium. If more than about one-half 45 of 1% of copper be added to such a chrome steel, the copper has a tendency to segregate, and to adversely affect the physical properties of the metal, especially its dynamic strength and resistance to impact. In steels of a higher chromium content, more than 50 one-half of 1% of copper may be added without this tendency, but apparently one-half of 1% of copper is a critical limit for steels having not over 2 or 3% of chromium.

55 While the amount of chromium may be increased above 1 or 1 1/4% and the amount of copper increased above .4 or .5% such additional amounts do not increase the beneficial effects sought for in ordinary steels. For example, .7 or .8% of copper does not 60 apparently give any more beneficial results than about .4% of copper, the extra copper apparently being more or less inert, and its addition involving needless expense. The extra copper is, if anything, deleterious, particularly for low chromium contents, on ac-

count of the tendency for the copper to segregate.

The chromium has the effect of increasing the hardness of the steel and its tensile strength, but without materially increasing 70 its dynamic strength. By "dynamic strength" is meant the resistance of the steel to repeated shocks, small stresses and vibrations. The addition of the copper increases the ductility and the dynamic strength of 75 the steel, while still preserving the increased tensile strength and hardness due to the chromium. The addition of the copper and chromium to steel, as herein specified, also increases the ratio of the elastic limit to the 80 ultimate strength. I have found that with the amounts of copper and chromium which I employ for ordinary steels, the chromium tends to make the steel less malleable, while the copper increases its malleability and the 85 two combined give a steel which has great tensile strength and hardness, but which can be rolled and forged.

In forming the alloy, sufficient carbon should be present to give the desired tensile 90 strength and hardness in combination with the chromium and copper. The carbon should in general be over .1% to be effective in imparting high tensile strength and hardness to the steel. The chromium and copper apparently react with the carbon and tend to maintain the carbon as hardening carbon and prevent its segregation as a cementite or graphite. This permits the alloy to be quenched more slowly than 95 plain carbon steel. The copper and chromium hold the carbon in its combined hardening form at an increased temperature. This is of considerable advantage in the making of tool or roll steel, which is subjected to heat, because the steel will not 100 soften in use at a temperature which would soften the plain carbon steel. The ability of the copper and chromium to hold the carbon in its hardening state is particularly 105 valuable in high carbon steels or high carbon cast iron, in that a high percentage of carbon may be kept in the hardening state 110 so as to form a very hard article.

The addition of the copper to the chromium steel makes the steel non-corrodible in all states, whether hardened or annealed or polished or rough, thus being a great improvement over the usual chromium steels which, while showing great resistance to 115 corrosion, when polished, will be corroded if the surface is rough.

In the above described ferrous alloys no reference is made to the presence of other elements, such as manganese, sulphur, etc., always present in steels and cast irons, as their presence to the usual extent does not interfere with the physical properties or non-corrosiveness of the described ferrous alloys.

The present invention is not limited to the exact proportions set forth, as its preferred embodiment, but may be otherwise embodied within the scope of the following claims.

I claim:

1. A ferrous alloy containing about .2 to .4% copper and .4 to 1% chromium together with carbon.
2. A ferrous alloy containing over .15% but less than .5% copper and between .3% and 3.5% chromium.
3. A ferrous alloy containing copper in appreciable amounts but less than .5% and

chromium in appreciable amounts but not over 3.5%. 15

4. A ferrous alloy consisting principally of iron and containing chromium in an appreciable amount, but less than 8% and copper over .15% but less than .5%.

5. A ferrous alloy containing about .2 to .4% copper and about .3 to 3.5% chromium together with carbon.

In testimony whereof I have hereunto set my hand.

BYRAMJI D. SAKLATWALLA.